

## UNITED STATES PATENT OFFICE

2,094,082

## DYEING OF CELLULOSIC MATERIALS

Leslie Paige Rendell and Harry Augustus Thomas, Blackley, Manchester, England, assignors to Imperial Chemical Industries Limited, a corporation of Great Britain

No Drawing. Application April 8, 1935, Serial No. 15,310. In Great Britain April 13, 1934

## 12 Claims.

(Cl. 8—5)

This invention relates to dyeing. More particularly it deals with a novel process for dyeing material of vegetable origin, such as textile fiber or non-fibrous material comprising cellulose or cellulose derivatives.

It is an object of this invention to provide a novel process of dyeing, whereby chrome dyestuffs, which have hitherto been applicable to animal fibers only, may be made available for dyeing vegetable materials. Other and further important objects of this invention will appear as the description proceeds.

In British Specification No. 398,175 is described a process wherein a textile material composed of cellulose, natural or regenerated, or of wool or other materials is treated before or after the dyeing operation with a dilute aqueous solution of certain heterocyclic ammonium salts, but the dyeing processes described relate only to those in which, on cellulosic materials, substantive and direct acid dyes are used.

In French Patent No. 725,637, wherein a similar process is described, it is stated that the improvement is applicable also to acetate silk. The dyestuffs, however, are again limited to those known as direct and acid dyestuffs.

We have now found that the invention may be extended also to chrome dyestuffs, such as have heretofore been applicable only to wool and other animal fibers.

More particularly, we have found that material of vegetable origin, such as cellulosic fiber, both natural and regenerated, or cellulose ethers and esters, may be endowed with an affinity for chrome dyestuffs, if treated with a quaternary ammonium salt, of the types mentioned in said patents.

By chrome dyestuffs, we are referring to such dyestuffs which are generally applied directly from a neutral or acid aqueous solution, and which are fixed upon the fiber by the aid of water-soluble chromates or bichromates. These latter may be present in the dyeing bath during the dyeing operation (the meta-chrome process), or they may be added to said bath after the dye has been exhausted (the after-chrome process). Or again, the fiber may be treated in a chromate bath first, and then dyed with the dyestuff (the chrome-mordant process).

We have further found that in lieu of the quaternary nitrogen compounds or ammonium salts mentioned in said patents, or in addition thereto if one so prefers, one may use phosphonium or sulfonium derivatives. In general, our invention is capable of operation with water-

soluble organic salts of inorganic acids, which have the property of ionizing in aqueous solution to give a long-chain, organic cation (positively charged ion) and an inorganic anion. In this respect the assistants applicable for our novel purpose may be contrasted with ordinary soaps, such as sodium stearate, palmitate or oleate, which upon ionization give a long-chain, organic anion and an inorganic cation. By the terms "inorganic acids" and "inorganic ions" in the preceding paragraph as well as in the claims below, we mean to cover and include polybasic inorganic acids or ions which have part of their acidity neutralized by organic radicals, as is illustrated by methyl-sulfuric acid which gives rise to the methosulfate ion.

According to the invention we treat ("mordant", so to speak) cellulose, regenerated cellulosic textile material, or cellulose ester or ether material with an aqueous solution of a quaternary ammonium, phosphonium or sulphonium salt, the molecule of which contains a saturated or unsaturated aliphatic chain of at least 10 carbon atoms which is free of water-solubilizing acid reacting substituents such as sulfo or carboxy, and we subsequently dye the material or print it if desired with a chrome dyestuff by the methods usually employed for dyeing or printing animal fibers with such dyestuffs.

The mordanting step may include padding, warming or boiling the textile material with an aqueous solution of the assistant, as is most convenient. The aqueous solution may vary in concentration within a wide range, say from  $\frac{1}{2}$  to 10% by weight of the assistant.

The chroming step may include the after-chrome, metachrome (chromate), or chrome-mordant processes, or modifications or combinations of these methods.

The effect of our novel process is to endow the fiber with an affinity for the dyestuffs in question or for the oxides of chromium or for both, and to produce dyeings of satisfactory fastness to washing and to light. The fastness to light of many of the dyeings so produced is of the same order as that obtained when the dyestuffs are applied as is customary to wool and other animal fibers. Other advantages of the invention are indicated below.

Examples of suitable salts for use according to the invention are: octadecyl-pyridinium bromide, the ester of oleic acid and N-hydroxyethyl-pyridinium chloride, the cetyl ether of N-hydroxy-methyl-pyridinium chloride, cetyl-trimethyl-ammonium chloride, dimethyl-dicetyl-ammecnium

bromide, cetyl-pyridinium bromide, cetyl-tri-methyl-ammonium bromide, octadecyl-trimethyl-ammonium methyl-sulphate, the trimethyl-ammonium methyl-sulphate of monostearyl-ethylene diamine, heptadecylamine hydrochloride, decylamine hydrochloride, dodecylamine hydrochloride, cetyl-dimethyl-sulphonium methyl-sulphate, benzyl-ethyl-dodecyl-sulphonium chloride, and benzyl-methyl-dodecyl sulphonium methyl-sulphate. It will be noted that all the above compounds are free of sulfo or carboxy groups in the cation portion of the molecule, thereby rendering the water-solubility of the compound more substantially dependent on the character of its anionic portion.

Some of the above are novel compounds, and are described more fully and claimed in co-pending applications Serial Nos. 611,236 and 28,013. Their general schemes of synthesis, however, 20 may be illustrated briefly by the following examples.

Dimethyl-dicetyl-ammonium bromide may be prepared by reacting one equivalent of dimethylamine and two equivalents of cetyl bromide. 25 Dimethyl-cetyl-sulphonium methyl-sulphate may be prepared by treating cetyl bromide with sodium hydrosulphide in alcohol, subjecting the mercaptan thus formed to an alkylation treatment with dimethyl sulphate and caustic soda, and 30 thereafter obtaining the salt by treatment with dimethyl sulphate alone. Benzylmethyldodecyl sulphonium methyl-sulphate is obtained by treating the mercaptan derived from dodecyl bromide with a mixture of sodium ethoxide and benzyl chloride and finally treating the resulting product with dimethyl sulphate.

Further examples of suitable assistants are the sulfonium compound obtainable by reacting dimethyl sulphate with 2-octadecyl-mercapto-benzothiazole (in turn obtainable by reacting octadecyl bromide with the sodium salt of 2-mercapto-benzothiazole); and quaternary phosphonium compounds such as cetyl-trimethyl-phosphonium bromide (obtainable by interacting trimethyl-phosphine and cetyl bromide) and dodecyl-trimethyl-phosphonium bromide (similarly made from dodecyl bromide and trimethyl-phosphine).

The invention is illustrated but not limited by 50 the following examples, in which the weight of substances employed in the dye-bath are expressed, as usual, as percentages of the weight of material to be dyed.

#### Example I

Viscose stockinette is mordanted at 90° C. by immersion for 1/2 hour in a 40:1 aqueous liquor containing 3.0% of cetyl-trimethyl-ammonium bromide. It is then thoroughly rinsed, and entered into a warm dye-bath containing 3.0% of the acid chrome dyestuff known as Solochrome Brown RH (Colour Index No. 98) and 3% of acetic acid and 10% of Glauber's salt. The temperature is gradually raised to 90-95° C. and after 1/2 hour, 2% of formic acid is added. Exhaustion of the dye-bath is satisfactory after a further 1/4 hour, and 1 1/2% of potassium dichromate is added as an aqueous solution. The shade is completely developed during 1/2-3/4 hour at 95° C. and is of good fastness to light and washing (particularly as regards non-staining of adjacent white cotton and viscose).

#### Example II

Viscose stockinette is mordanted by immersion

at 90-95° C. for 1/2 hour in a 40:1 aqueous liquor containing 3% of cetyl-pyridinium bromide, and is then thoroughly rinsed and entered at 50° C. into a dye bath prepared with 3% of the azo acid chrome dyestuff known as Solochrome Brown MG (Colour Index No. 101), 2% of potassium dichromate and 8% of ammonium sulphate and made slightly alkaline with ammonia. The temperature is gradually increased to 95° C. and after 3/4 hour the bath is exhausted satisfactorily without any addition of acid. A full brown shade is obtained of good fastness to washing and light.

#### Example III

Viscose stockinette is mordanted by immersion for 1/2 hour at 95° C. in a 40:1 aqueous liquor containing 3% of cetyl-pyridinium bromide and is then rinsed and entered into a chrome mordanting bath containing 3% of potassium dichromate and 2 1/2% of cream of tartar. The temperature is maintained at 95° C. for 1/2 hour, and the material is then rinsed and entered into a warm dye-bath containing 3.0% of the acid-chrome dyestuff known as Solochrome Orange GR (Colour Index Supplement, page 52). The temperature is gradually raised to 95° C. and after 1/2 hour, 1% of acetic acid is added. The bath is exhausted satisfactorily and the orange shade obtained is of good fastness to washing and light.

#### Example IV

Viscose stockinette is mordanted with 3% of cetyl-pyridinium bromide and afterwards with reduced bichrome as described under Example III, and is then rinsed and dyed with 3% of the acid chrome dyestuffs known as Solochrome Red ERS. After dyeing at 90° C. for 1/2 hour, 1% of acetic acid is added and dyeing continued for a further 3/4 hour when 1% of potassium bichromate is added as an aqueous solution, and dyeing continued for a further 20 minutes.

A full red shade is obtained of good fastness to washing.

#### Example V

Cotton piece goods is mordanted with 3% of dimethyl-dicetyl-ammonium bromide at 90° C. for 1/2 hour in a 40:1 aqueous liquor, and is then rinsed and entered at 50-60° C. in a dye-bath containing 3% of the acid chrome dyestuff known as Solochrome Brown MG (Colour Index No. 101), and 2% of acetic acid. The temperature is raised to 95° C. and after dyeing for 1/2 hour a further 1% of acetic acid is added. The bath is well exhausted after a further 10 minutes, when 1% of bichrome is added, and afterchroming performed for 1/2 hour at 95° C.

The brown shade obtained is of very good fastness to washing.

#### Example VI

Viscose stockinette is mordanted for 1/2 hour at 90° C. with 3% of octadecyl-trimethyl-ammonium methyl-sulphate in a 40:1 aqueous liquor, and is then thoroughly rinsed and entered at 60° C. into a dye-bath containing 3% of the azo-acid chrome dyestuff known as Solochrome Brown MG (Colour Index No. 101) and 2% of acetic acid. The temperature is raised to 95° C. and after dyeing has been in progress for 1/2 hour, a further 1% of acetic acid is added. Exhaustion is complete during a further 10 minutes, when 1 1/2% of bichrome is added, and afterchroming is performed at 95° C. for 1/2 hour when

a full brown shade of very good fastness to washing and light is obtained.

*Example VII*

5 Viscose stockinette is mordanted with 3.0% of dimethyl-cetyl-sulphonium methyl-sulphate by immersion for  $\frac{1}{2}$  hour at 90-95° C. in the aqueous solution. It is then dyed a red shade by immersion in an aqueous liquor containing 3% 10 of Solochrome Red 6B (I. C. I. Dyestuffs Sales Circular S. C. 110), 3.0% of acetic acid and 10% of Glauber's salt, calculated on the weight of material. After  $\frac{1}{2}$  hour's dyeing at 90-95° C., an addition of 1% of formic acid is made, and after 15 a further  $\frac{1}{4}$  hour a further addition of 1%. Afterchroming is then performed by addition of 1% of potassium dichromate and heating at 90-95° C. for  $\frac{1}{2}$  hour.

The shade obtained possesses very good fastness to washing and light.

*Example VIII*

25 Viscose stockinette mordanted as above with 3% of benzyl - methyl - dodecyl - sulphonium methyl-sulphate is dyed by the afterchrome process as described in Examples IV-VI with 3% of Solochrome Yellow C (Colour Index No. 343). 3% of acetic acid and 10% of Glauber's salt are present during the dyeing and the bath is exhausted with the addition of 2% of formic acid. Afterchroming is performed with the addition of 1% of potassium bichromate.

30 A yellow shade of good fastness properties is obtained.

*Example IX*

40 Acetate artificial silk stockinette fabric is mordanted for half an hour at 75° C. in an aqueous solution of 3% of octadecyl-trimethyl-ammonium methyl-sulphate, the amount of liquor being 40 times that of the material. The fabric is well rinsed in warm water and then put into a dye-bath (at 50° C.) containing 3.0% of the chrome dyestuff known as Solochrome Brown M (Colour Index No. 101), and 2% of acetic acid. The temperature is increased to 80° C. and after half an hour a further 1% of acetic acid is added, followed by 1½% of sodium bichromate after a further 10 minutes.

50 After chroming for half an hour at 80-85° C. a medium brown shade of good fastness to washing and light is obtained. The dye liquor is exhausted very satisfactorily.

*Example X*

55 Acetate artificial silk stockinette fabric is mordanted for half an hour at 70-75° C. in an aqueous solution containing 3% of cetyl-pyridinium bromide, and is then dyed with 2% of the 60 chrome dyestuff known as Solochrome Yellow C (Colour Index No. 343), by the afterchrome process as described in Example IX. The dye liquor is well exhausted, and a good yellow shade is obtained.

*Example XI*

65 Acetate artificial silk stockinette is mordanted with 3% of cetyl-pyridinium bromide as in Example X, and is dyed by the metachrome process with 3.0% of the chrome dyestuff known as Solochrome Yellow WN (Colour Index No. 36). 70 2% of sodium bichromate and 4% of ammonium sulphate is employed in the dye-bath, and dyeing is performed at 80° C. for three quarters of an hour. A good yellow shade is obtained.

*Example XII*

Acetate artificial silk stockinette fabric is mordanted with 3% of dimethyl-dicetyl-ammonium bromide at 70-75° C. for half an hour, from an aqueous solution of the quaternary ammonium compound. The mordanted material is well rinsed in water and then heated for three quarters of an hour at 75-80° C. in an aqueous solution containing 3% of potassium bichromate and 3% of cream of tartar. The chrome mordanted material is then rinsed and entered at 50° C. into a dye-bath containing 4% of the chrome dye-stuff known as Solochrome Brown NH (Colour Index No. 105). The temperature is increased to 80° C. and after half an hour 1% of sulphuric acid and 1% of potassium bichromate (as concentrated aqueous solution) are added in order to develop the shade fully.

A medium brown shade is obtained.

5

10

15

20

25

30

35

*Example XIII*

Glycol-cellulose is mordanted by treatment for half an hour at 90-95° C. in an aqueous solution of cetyl-pyridinium bromide containing 3% of the quaternary ammonium compound on the weight of glycol-cellulose. The material is then rinsed and dyed by the afterchrome process at 90-95° C. with 3% of the chrome dyestuff known as Solochrome Cyanine R (Colour Index No. 722), 30 with the addition of 3% of acetic acid to the dye-bath and 2% of formic acid for exhaustion. Afterchroming is performed with the addition of 1½% of sodium bichromate when a full bright blue shade is obtained of excellent fastness to 35 washing.

*Example XIV*

Ethylcellulose powder is mordanted at 90° C. from an aqueous solution containing 3% of cetyl-pyridinium bromide, by treatment for half an hour. It is then filtered off, washed with water and dyed by the afterchrome process with 3% of the chrome dyestuff known as Solochrome Azurine B (Colour Index No. 720). The temperature is 45 maintained at 90-95° C. during the dyeing and chroming operations. 3% of acetic acid and 1% of formic acid are employed in the dye-bath. The dark blue powder obtained may be dissolved in acetone or ethyl alcohol to give a deep blue 50 solution of high tintorial value from which blue films can be obtained.

*Example XV*

Ethyl cellulose powder mordanted as described 55 in Example XIV is dyed by the afterchrome process at 90-95° C. with 3% of the chrome dyestuff known as Solochrome Yellow C (Colour Index 343). A dark yellow powder is obtained which may be dissolved in acetone or alcohol to give 60 a deep yellow solution which yields a yellow film.

*Example XVI*

Acetate artificial silk stockinette is mordanted at 75° C. for half an hour from an aqueous solution containing 3% of dimethyl-cetyl-sulphonium methyl-sulphate, and is then rinsed in water and dyed by the afterchrome process at 75-80° C. with 3% of the chrome dyestuff known as Solochrome Yellow C (Colour Index No. 343), 3% of acetic acid, and 1% of sulphuric acid are employed in the dye-bath, and 1½% of potassium bichromate is employed for afterchroming. A yellow shade of 70 medium depth and good fastness to washing is obtained.

65

70

75

*Example XVII*

Acetate artificial silk stockinette mordanted with 3% of dimethyl-cetyl-sulphonium methylsulphate, as described in Example XVI, is dyed by the afterchrome process at 75-80° C. with 3% of chrome dyestuff known as Solochrome Cyanine R (Colour Index No. 722) with addition of 3% of acetic acid and 1% of sulphuric acid to the dye-bath; 1½% of potassium bichromate being employed for afterchroming.

The bright blue shade obtained is of good fastness to washing.

*Example XVIII*

Viscose stockinette is mordanted by immersion at 95° C. for ½ hour in a 40:1 aqueous liquor containing 3% heptadecylamine hydrochloride. It is then rinsed and dyed by immersion in a dye-liquor set with 3% of the acid-chrome dyestuff known as Gallo-cyanine BD (Colour Index 883) and 3% of acetic acid with 10% of Glauber's salt. The temperature is gradually raised to 90° C.-95° C. After ½ hour at this temperature 2% of sulphuric acid is added and a further ¼ hour at 90° C.-95° C. is then sufficient to ensure complete exhaustion. At this stage 2% of potassium dichromate is added and the shade fully developed in ½ hour to ¾ hour. The resultant shade is a strong navy blue of excellent fastness to light and washing.

*Example XIX*

Viscose stockinette is mordanted by immersion for ½ hour at 90°-95° C. in a 40:1 aqueous liquor containing 3% of heptadecylamine hydrochloride. It is then thoroughly rinsed and immersed in a warm dye-bath containing 3% of the acid chrome dyestuff known as Solochrome Brown MG (Colour Index No. 101) and 3% acetic acid with 10% Glauber's salt. The temperature is slowly raised to 90° C.-95° C. After ½ hour at this temperature a further addition of 2% of sulphuric acid is made to the dye-bath to ensure complete exhaustion which is obtained after a further ¼ hour. 2% of potassium dichromate is then added and the shade fully developed after ½-¾ hour at 90-95° C. The bright brown shade obtained is of excellent fastness to light and washing.

*Example XX*

Acetate silk stockinette is mordanted by immersion at 75° C. in a 40:1 aqueous liquor containing 3% of heptadecylamine hydrochloride for ½ hour. It is then rinsed and immersed in a warm dye-bath set with 3% of the acid chrome dyestuff known as Solochrome Brown MG (Colour Index No. 101) with 3% acetic and 10% Glauber's salt. The temperature is slowly raised to 75° C. and after ½ hour at 75° C. 2% of sulphuric acid is added to complete the exhaustion of the dyebath, which is satisfactory after a further ¼ hour. At this stage 2% potassium dichromate is added and after a further ½ hour the shade is fully developed. A bright brown shade is obtained which is of good fastness to light and washing.

In place of heptadecylamine hydrochloride there can be used other long chain amines such as decylamine hydrochloride or dodecylamine hydrochloride.

It will be understood that the details of procedure may be varied within wide limits without departing from the spirit of this invention.

Thus, while we have indicated in each of the above examples a 3% solution of the mordanting organic salt and used it in a ratio of 40:1 compared to the weight of the cellulosic material, these figures have been adhered to merely as a standard for comparison. Various other ratios may obviously be employed, and the concentration may vary within wide limits, say from ½% to 10% depending on the intensity of effect desired.

Similarly, although in the above examples we worked at temperatures from 70 to 95° C., any other convenient temperature between room temperature and boiling water may be employed. As in the case of mordanting with metallic oxides, the application of the mordant to the fiber may be effected by padding, spraying, impregnating or immersion.

Many other variations and modifications will be obvious to those skilled in the art.

We claim:

1. A process for coloring textile fiber of cellulosic origin with acid-chrome dyestuffs normally applicable to wool only, which comprises warming said fiber in an aqueous bath of an organic salt selected from the group consisting of long-chain ammonium, phosphonium, and sulfonium salts of strong mineral acids, the long-chain comprising an aliphatic chain of at least 10 carbon atoms, and then dyeing said fiber with an acid-chrome dyestuff by one of the methods generally applicable with dyestuffs of this class.

2. A process for colouring textile material of cellulosic origin, which comprises mordanting the same with an aqueous solution of a water-soluble organic salt selected from the group consisting of organic quaternary ammonium, quaternary phosphonium and ternary sulfonium compounds which contain at least one aliphatic chain of not less than 10 carbon atoms, and then dyeing said material with an acid-chrome dyestuff for wool in the same manner as wool would normally be dyed with a dyestuff of the same class.

3. The process which comprises mordanting textile fiber comprising cellulose with an aqueous solution of an organic salt selected from the group consisting of quaternary ammonium, quaternary phosphonium and ternary sulfonium derivatives of strong mineral acids, the salt containing at least one aliphatic chain of not less than 10 carbon atoms and which is free of water-solubilizing acid reacting substituents, and then dyeing said fiber with an acid-chrome dyestuff, by one of the processes known as the chrome-mordant, metachrome, and afterchrome methods.

4. The process which comprises mordanting material comprising cellulose acetate with an aqueous solution of an organic salt selected from the group consisting of quaternary ammonium, quaternary phosphonium and ternary sulfonium derivatives of strong mineral acids, the salt containing at least one aliphatic chain of not less than 10 carbon atoms but free of sulfo or carboxy groups, and then dyeing said material with an acid-chrome dyestuff by one of the processes known as the chrome-mordant, metachrome, and afterchrome methods.

5. The process which comprises mordanting cellulosic fiber with an aqueous solution of an organic ammonium compound capable of dissociating and yielding a positively charged organic ion comprising a long-chain aliphatic radical of not less than 10 carbon atoms and being free of water-solubilizing acid reacting substituents, and then treating the fiber in optional

time relation with an aqueous solution of an acid-chrome dye and an aqueous solution of a chroming agent.

6. A process for colouring textile material of cellulosic origin, which comprises mordanting the same with an aqueous solution of an organic ammonium salt selected from the group consisting of organic ammonium halides and organic ammonium methyl-sulfates, the organic radical of which contains at least one straight chain aliphatic radical of not less than 10 carbon atoms, and then dyeing said material with an acid-chrome dyestuff for wool in the same manner as wool would normally be dyed with a dyestuff of the same class.

7. A process for colouring textile material of cellulosic origin, which comprises mordanting the same with an aqueous solution of an organic quaternary ammonium halide which contains in the nitrogen atom at least one straight chain aliphatic radical of from 10 to 18 carbon atoms, said aliphatic radical being free of water-solubilizing acid reacting substituents, and then dyeing said material with an acid-chrome dyestuff, by one of the processes known as the chrome-mordant, metachrome, and afterchrome methods.

8. A process for colouring textile material of cellulosic origin, which comprises mordanting the same with an aqueous solution of a primary alkyl ammonium halide the alkyl portion of which contains a straight chain aliphatic radical of from 10 to 18 carbon atoms but no water-solubilizing acid reacting substituents, and then dyeing said material with an acid-chrome dyestuff, by one of

the processes known as the chrome-mordant, metachrome, and afterchrome methods.

9. A process for colouring textile material of cellulosic origin, which comprises mordanting the same with an aqueous solution of an alkyl pyridinium halide the alkyl portion of which contains a straight chain aliphatic radical of from 10 to 18 carbon atoms, and then dyeing said material with an acid-chrome dyestuff, by one of the processes known as the chrome-mordant, metachrome, and afterchrome methods. 5

10. A process for colouring textile material of cellulosic origin, which comprises mordanting the same with an aqueous solution of octadecyl-trimethyl-ammonium methyl-sulfate, and then 15 dyeing said material with an acid-chrome dyestuff, by one of the processes known as the chrome-mordant, metachrome, and afterchrome methods.

11. A process for colouring textile material of cellulosic origin, which comprises mordanting the same with an aqueous solution of cetyl-trimethyl-ammonium bromide, and then dyeing said material with an acid-chrome dyestuff, by one of the processes known as the chrome-mordant, metachrome, and afterchrome methods. 20 25

12. A process for colouring textile material of cellulosic origin, which comprises mordanting the same with an aqueous solution of cetyl pyridinium bromide, and then dyeing said material with an acid-chrome dyestuff, by one of the processes known as the chrome-mordant, metachrome, and afterchrome methods. 30

LESLIE PAIGE RENDELL. 35  
HARRY AUGUSTUS THOMAS.